



US008334243B2

(12) **United States Patent**  
**Guevremont et al.**

(10) **Patent No.:** **US 8,334,243 B2**  
(45) **Date of Patent:** **Dec. 18, 2012**

(54) **LUBRICANT COMPOSITIONS CONTAINING A FUNCTIONALIZED DISPERSANT FOR IMPROVED SOOT OR SLUDGE HANDLING CAPABILITIES**

(75) Inventors: **Jeffrey M. Guevremont**, Richmond, VA (US); **Jason A. Lagona**, Richmond, VA (US)

(73) Assignee: **Afton Chemical Corporation**, Richmond, VA (US)

(\*) Notice: Subject to any disclaimer, the term of this patent is extended or adjusted under 35 U.S.C. 154(b) by 160 days.

(21) Appl. No.: **13/049,117**

(22) Filed: **Mar. 16, 2011**

(65) **Prior Publication Data**

US 2012/0234287 A1 Sep. 20, 2012

(51) **Int. Cl.**

*C10M 133/38* (2006.01)  
*C10M 133/44* (2006.01)  
*C10M 133/48* (2006.01)

(52) **U.S. Cl.** ..... **508/231; 508/268; 508/296**

(58) **Field of Classification Search** ..... **508/231, 508/268, 296**

See application file for complete search history.

(56) **References Cited**

U.S. PATENT DOCUMENTS

4,259,194 A 3/1981 DeVries et al.  
4,259,195 A 3/1981 King et al.  
4,261,843 A 4/1981 King et al.  
4,263,152 A 4/1981 King et al.  
4,265,773 A 5/1981 DeVries et al.  
4,272,387 A 6/1981 King et al.

|                 |         |                    |
|-----------------|---------|--------------------|
| 4,283,295 A     | 8/1981  | deVries et al.     |
| 4,285,822 A     | 8/1981  | deVries et al.     |
| 4,702,850 A     | 10/1987 | Gutierrez et al.   |
| 4,867,890 A     | 9/1989  | Colclough et al.   |
| 4,943,672 A     | 7/1990  | Hamner et al.      |
| 5,882,505 A     | 3/1999  | Wittenbrink et al. |
| 6,013,171 A     | 1/2000  | Cook et al.        |
| 6,080,301 A     | 6/2000  | Berlowitz et al.   |
| 6,096,940 A     | 8/2000  | Wittenbrink et al. |
| 6,103,099 A     | 8/2000  | Wittenbrink et al. |
| 6,165,949 A     | 12/2000 | Berlowitz et al.   |
| 6,180,575 B1    | 1/2001  | Nipe               |
| 6,300,291 B1    | 10/2001 | Hartley et al.     |
| 6,548,458 B2    | 4/2003  | Loper              |
| 6,723,685 B2    | 4/2004  | Hartley et al.     |
| 7,214,649 B2    | 5/2007  | Loper et al.       |
| 7,576,161 B2    | 8/2009  | Stokes et al.      |
| 2004/0266630 A1 | 12/2004 | George et al.      |
| 2008/0194441 A1 | 8/2008  | Kawata et al.      |
| 2008/0274922 A1 | 11/2008 | Yagishita          |
| 2010/0249001 A1 | 9/2010  | Storey et al.      |

FOREIGN PATENT DOCUMENTS

WO 9406897 3/1994  
WO WO 2009051216 A1 \* 4/2009

\* cited by examiner

*Primary Examiner* — Prem C Singh

*Assistant Examiner* — Taiwo Oladapo

(74) *Attorney, Agent, or Firm* — Luedeka Neely Group, P.C.

(57) **ABSTRACT**

A crankcase lubricant composition, method for improving the soot or sludge handling capability of a crankcase lubricant composition and a method of operating an engine on a crankcase lubricant composition. The lubricant composition includes a base oil and a reaction product of mono-succinimide dispersant and an acidic compound containing two or more pyrrole groups.

**19 Claims, No Drawings**

**LUBRICANT COMPOSITIONS CONTAINING  
A FUNCTIONALIZED DISPERSANT FOR  
IMPROVED SOOT OR SLUDGE HANDLING  
CAPABILITIES**

**TECHNICAL FIELD**

The disclosure relates to lubricant compositions and in particular to additives for improving the soot or sludge handling characteristics of a crankcase lubricant composition.

**BACKGROUND AND SUMMARY**

Crankcase lubricant compositions may be selected to provide an increased engine protection while providing an increase in fuel economy and reduced emissions. However, in order to achieve benefits of improved fuel economy and reduced emissions, a balance between engine protection and lubricating properties is required for the lubricant composition. For example, an increase in the amount of friction modifiers may be beneficial for fuel economy purposes but may lead to reduced ability of the lubricant composition to handle water. Likewise, an increase in the amount of anti-wear agent in the lubricant may provide improved engine protection against wear but may be detrimental to catalyst performance for reducing emissions. Accordingly, there is a need for improved lubricant compositions that are suitable for meeting or exceeding currently proposed and future lubricant performance standards.

With regard to the foregoing, embodiments of the disclosure provide a crankcase lubricant composition, method for improving the soot or sludge handling capability of a crankcase lubricant composition and a method of operating an engine on a crankcase lubricant composition. The lubricant composition includes a base oil and a reaction product of mono-succinimide dispersant and an acidic compound containing two or more pyrrole groups.

An embodiment of the disclosure provides a method for improving the soot or sludge handling capability of a crankcase lubricant for an engine composition. The method includes formulating a lubricant composition for the engine with a base oil and a reaction product of a monosuccinimide dispersant and an acidic compound containing at least two pyrrole groups. The engine is operated with the crankcase lubricant to provide the improved soot and sludge handling capabilities.

A further embodiment of the disclosure provides a method for operating an engine. The method includes formulating a crankcase lubricant for the engine having a base oil and a lubricant additive package including a reaction product of a monosuccinimide dispersant and an acidic compound containing at least two pyrrole groups. The engine is operated with the crankcase lubricant.

Another embodiment of the disclosure provides a dispersant for a crankcase lubricant comprising a reaction product of monosuccinimide dispersant and an acidic compound containing at least two pyrrole groups.

An unexpected advantage of the use of a dispersant derivative provides improved soot or sludge handling capabilities to a lubricant. Such capabilities may be achieved with substantially less dispersant compared to a lubricant composition containing a conventional dispersant. A further advantage of the use of the dispersant derivative described herein is that since less dispersant is required to achieve comparable soot or sludge handling capabilities, lubricant compositions containing the dispersant may have greater seal compatibility and lower lead corrosion.

The following definitions of terms are provided in order to clarify the meanings of certain terms as used herein.

As used herein, the terms "oil composition," "lubrication composition," "lubricating oil composition," "lubricating oil," "lubricant composition," "lubricating composition," "fully formulated lubricant composition," and "lubricant" are considered synonymous, fully interchangeable terminology referring to the finished lubrication product comprising a major amount of a base oil plus a minor amount of an additive composition.

As used herein, the terms "additive package," "additive concentrate," and "additive composition" are considered synonymous, fully interchangeable terminology referring the portion of the lubricating composition excluding the major amount of base oil stock mixture.

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having predominantly hydrocarbon character. Examples of hydrocarbyl groups include:

- (1) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical);
- (2) substituted hydrocarbon substituents, that is, substituents containing non-hydrocarbon groups which, in the context of this invention, do not alter the predominantly hydrocarbon substituent (e.g., halo (especially chloro and fluoro), hydroxy, alkoxy, mercapto, alkylmercapto, nitro, nitroso, and sulfoxo);
- (3) hetero substituents, that is, substituents which, while having a predominantly hydrocarbon character, in the context of this invention, contain other than carbon in a ring or chain otherwise composed of carbon atoms. Heteroatoms include sulfur, oxygen, nitrogen, and encompass substituents such as pyridyl, furyl, thieryl, and imidazolyl. In general, no more than two, for example, no more than one, non-hydrocarbon substituent will be present for every ten carbon atoms in the hydrocarbyl group; typically, there will be no non-hydrocarbon substituents in the hydrocarbyl group.

As used herein, the term "percent by weight", unless expressly stated otherwise, means the percentage the recited component represents to the weight of the entire composition.

The terms "oil-soluble" or "dispersible" used herein do not necessarily indicate that the compounds or additives are soluble, dissolvable, miscible, or capable of being suspended in the oil in all proportions. The foregoing terms do mean, however, that they are, for instance, soluble or stably dispersible in oil to an extent sufficient to exert their intended effect in the environment in which the oil is employed. Moreover, the additional incorporation of other additives may also permit incorporation of higher levels of a particular additive, if desired.

Crankcase lubricating oils of the present disclosure may be formulated by the addition of one or more additives, as described in detail below, to an appropriate base oil formulation. The additives may be combined with a base oil in the form of an additive package (or concentrate) or, alternatively, may be combined individually with a base oil. The fully formulated crankcase lubricant may exhibit improved performance properties, based on the additives added and their respective proportions.

Additional details and advantages of the disclosure will be set forth in part in the description which follows, and/or may be learned by practice of the disclosure. The details and advantages of the disclosure may be realized and attained by means of the elements and combinations particularly pointed out in the appended claims.

It is to be understood that both the foregoing general description and the following detailed description are exemplary and explanatory only and are not restrictive of the disclosure, as claimed.

#### DESCRIPTION OF THE EXEMPLARY EMBODIMENTS

The present disclosure will now be described in the more limited aspects of embodiments thereof, including various examples of the formulation and use of the present disclosure. It will be understood that these embodiments are presented solely for the purpose of illustrating the invention and shall not be considered as a limitation upon the scope thereof.

Crankcase lubricant compositions are used in vehicles containing spark ignition and compression ignition engines. Such engines may be used in automotive and truck applications and may be operated on fuels including, but not limited to, gasoline, diesel, alcohol, compressed natural gas, and the like. The disclosure is directed specifically to crankcase lubricants, and more particularly to automotive crankcase lubricants that meet or exceed the proposed ILSAC GF-5 lubricant standards.

##### Base Oil

Base oils suitable for use in formulating crankcase lubricant compositions may be selected from any of suitable synthetic or natural oils or mixtures thereof. Natural oils may include animal oils and vegetable oils (e.g., castor oil, lard oil) as well as mineral lubricating oils such as liquid petroleum oils and solvent treated or acid-treated mineral lubricating oils of the paraffinic, naphthenic or mixed paraffinic-naphthenic types. Oils derived from coal or shale may also be suitable. The base oil typically may have a viscosity of about 2 to about 15 cSt or, as a further example, about 2 to about 10 cSt at 100° C. Further, an oil derived from a gas-to-liquid process is also suitable.

Suitable synthetic base oils may include alkyl esters of dicarboxylic acids, polyglycols and alcohols, poly-alpha-olefins, including polybutenes, alkyl benzenes, organic esters of phosphoric acids, and polysilicone oils. Synthetic oils include hydrocarbon oils such as polymerized and interpolymerized olefins (e.g., polybutylenes, polypropylenes, propylene isobutylene copolymers, etc.); poly(1-hexenes), poly(1-octenes), poly(1-decenes), etc. and mixtures thereof; alkyl-benzenes (e.g., dodecylbenzenes, tetradecylbenzenes, di-nonylbenzenes, di-(2-ethylhexyl)benzenes, etc.); polyphenyls (e.g., biphenyls, terphenyl, alkylated polyphenyls, etc.); alkylated diphenyl ethers and alkylated diphenyl sulfides and the derivatives, analogs and homologs thereof and the like.

Alkylene oxide polymers and interpolymers and derivatives thereof where the terminal hydroxyl groups have been modified by esterification, etherification, etc., constitute another class of known synthetic oils that may be used. Such oils are exemplified by the oils prepared through polymerization of ethylene oxide or propylene oxide, the alkyl and aryl ethers of these polyoxyalkylene polymers (e.g., methyl-polyisopropylene glycol ether having an average molecular weight of about 1000, diphenyl ether of polyethylene glycol having a molecular weight of about 500-1000, diethyl ether of polypropylene glycol having a molecular weight of about

1000-1500, etc.) or mono- and polycarboxylic esters thereof, for example, the acetic acid esters, mixed C<sub>3</sub>-C<sub>8</sub> fatty acid esters, or the C<sub>13</sub> oxo-acid diester of tetraethylene glycol.

Another class of synthetic oils that may be used includes the esters of dicarboxylic acids (e.g., phthalic acid, succinic acid, alkyl succinic acids, alkenyl succinic acids, maleic acid, azelaic acid, suberic acid, sebacic acid, fumaric acid, adipic acid, linoleic acid dimer, malonic acid, alkyl malonic acids, alkenyl malonic acids, etc.) with a variety of alcohols (e.g., butyl alcohol, hexyl alcohol, dodecyl alcohol, 2-ethylhexyl alcohol, ethylene glycol, diethylene glycol monoether, propylene glycol, etc.) Specific examples of these esters include dibutyl adipate, di(2-ethylhexyl)sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, the complex ester formed by reacting one mole of sebacic acid with two moles of tetraethylene glycol and two moles of 2-ethylhexanoic acid and the like.

Esters useful as synthetic oils also include those made from C<sub>5</sub> to C<sub>12</sub> monocarboxylic acids and polyols and polyol ethers such as neopentyl glycol, trimethylol propane, pentaerythritol, dipentaerythritol, tripentaerythritol, etc.

Hence, the base oil used which may be used to make the crankcase lubricant compositions as described herein may be selected from any of the base oils in Groups I-V as specified in the American Petroleum Institute (API) Base Oil Interchangeability Guidelines. Such base oil groups are as follows:

TABLE 1

| Base Oil Group <sup>1</sup> | Sulfur (wt %) | Saturates (wt %)                       |     | Viscosity Index |
|-----------------------------|---------------|----------------------------------------|-----|-----------------|
| Group I                     | >0.03         | And/or                                 | <90 | 80 to 120       |
| Group II                    | ≤0.03         | And                                    | ≥90 | 80 to 120       |
| Group III                   | ≤0.03         | And                                    | ≥90 | ≥120            |
| Group IV                    |               | all polyalphaolefins (PAOs)            |     |                 |
| Group V                     |               | all others not included in Groups I-IV |     |                 |

<sup>1</sup>Groups I-III are mineral oil base stocks.

The base oil may contain a minor or major amount of a poly-alpha-olefin (PAO). Typically, the poly-alpha-olefins are derived from monomers having from about 4 to about 30, or from about 4 to about 20, or from about 6 to about 16 carbon atoms. Examples of useful PAOs include those derived from octene, decene, mixtures thereof, and the like. PAOs may have a viscosity of from about 2 to about 15, or from about 3 to about 12, or from about 4 to about 8 cSt at 100° C. Examples of PAOs include 4 cSt at 100° C. poly-alpha-olefins, 6 cSt at 100° C. poly-alpha-olefins, and mixtures thereof. Mixtures of mineral oil with the foregoing poly-alpha-olefins may be used.

The base oil may be an oil derived from Fischer-Tropsch synthesized hydrocarbons. Fischer-Tropsch synthesized hydrocarbons are made from synthesis gas containing H<sub>2</sub> and CO using a Fischer-Tropsch catalyst. Such hydrocarbons typically require further processing in order to be useful as the base oil. For example, the hydrocarbons may be hydroisomerized using processes disclosed in U.S. Pat. Nos. 6,103,099 or 6,180,575; hydrocracked and hydroisomerized using processes disclosed in U.S. Pat. Nos. 4,943,672 or 6,096,940; dewaxed using processes disclosed in U.S. Pat. No. 5,882,505; or hydroisomerized and dewaxed using processes disclosed in U.S. Pat. Nos. 6,013,171; 6,080,301; or 6,165,949.

Unrefined, refined, and rerefined oils, either natural or synthetic (as well as mixtures of two or more of any of these) of

the type disclosed hereinabove can be used in the base oils. Unrefined oils are those obtained directly from a natural or synthetic source without further purification treatment. For example, a shale oil obtained directly from retorting operations, a petroleum oil obtained directly from primary distillation or ester oil obtained directly from an esterification process and used without further treatment would be an unrefined oil. Refined oils are similar to the unrefined oils except they have been further treated in one or more purification steps to improve one or more properties. Many such purification techniques are known to those skilled in the art such as solvent extraction, secondary distillation, acid or base extraction, filtration, percolation, etc. Rerefined oils are obtained by processes similar to those used to obtain refined oils applied to refined oils which have been already used in service. Such rererefined oils are also known as reclaimed or reprocessed oils and often are additionally processed by techniques directed to removal of spent additives, contaminants, and oil breakdown products.

The base oil may be combined with an additive composition as disclosed in embodiments herein to provide a crankcase lubricant composition. Accordingly, the base oil may be present in the crankcase lubricant composition in an amount ranging from about 50 wt % to about 95 wt % based on a total weight of the lubricant composition.

#### Metal-Containing Detergents

Embodiments of the present disclosure may also comprise at least one metal detergent. Detergents generally comprise a polar head with a long hydrophobic tail where the polar head comprises a metal salt of an acidic organic compound. The salts may contain a substantially stoichiometric amount of the metal, in which case they are usually described as normal or neutral salts, and would typically have a total base number or TBN (as measured by ASTM D2896) of from about 0 to less than about 150. Large amounts of a metal base may be included by reacting an excess of a metal compound such as an oxide or hydroxide with an acidic gas such as carbon dioxide. The resulting overbased detergent comprises micelles of neutralized detergent surrounding a core of inorganic metal base (e.g., hydrated carbonates). Such overbased detergents may have a TBN of about 150 or greater, such as from about 150 to about 450 or more.

Detergents that may be suitable for use in the present embodiments include oil-soluble overbased sulfonates, phenates, sulfurized phenates, and salicylates of a metal, particularly the alkali or alkaline earth metals, e.g., sodium, potassium, lithium, calcium, and magnesium. More than one metal may be present, for example, both calcium and magnesium. Mixtures of calcium and/or magnesium with sodium may also be suitable. Suitable metal detergents may be overbased calcium or magnesium sulfonates having a TBN of from 100 to 450 TBN, overbased calcium or magnesium phenates or sulfurized phenates having a TBN of from 100 to 450, and overbased calcium or magnesium salicylates having a TBN of from 130 to 350. Mixtures of such salts may also be used.

The metal-containing detergent may be present in a lubricating composition in an amount of from about 0.5 wt % to about 5 wt %. As a further example, the metal-containing detergent may be present in an amount of from about 1.0 wt % to about 3.0 wt %. The metal-containing detergent may be present in a lubricating composition in an amount sufficient to provide from about 500 to about 5000 ppm alkali and/or alkaline earth metal to the lubricant composition based on a total weight of the lubricant composition. As a further example, the metal-containing detergent may be present in a lubricating composition in an amount sufficient to provide from about 1000 to about 3000 ppm alkali and/or alkaline earth metal.

#### Dispersant Derivatives

According to embodiments of the disclosure, the dispersant may be a reaction product of mono-succinimide dispersant and an acidic compound containing pyrrole groups. The mono-succinimide dispersant may be derived from a polyalkenyl or hydrocarbyl-substituted succinic acid or anhydride. In an aspect of the disclosed embodiments, the polyalkenyl or hydrocarbyl substituents of the hydrocarbyl-substituted succinic acids or anhydrides may be derived from butene polymers, for example polymers of isobutylene. Suitable polyisobutenes for use herein include those formed from polyisobutylene or highly reactive polyisobutylene having at least about 60%, such as about 70% to about 90% and above, terminal vinylidene content. Suitable polyisobutenes may include those prepared using  $\text{BF}_3$  catalysts. The average number molecular weight of the polyalkenyl substituent may vary over a wide range, for example from about 100 to about 5000, such as from about 500 to about 5000, as determined by GPC as described above.

In making the mono-succinimide dispersant according to the disclosure, carboxylic reactants other than maleic anhydride may be used such as maleic acid, fumaric acid, malic acid, tartaric acid, itaconic acid, itaconic anhydride, citraconic acid, citraconic anhydride, mesaconic acid, ethylmaleic anhydride, dimethylmaleic anhydride, ethylmaleic acid, dimethylmaleic acid, hexylmaleic acid, and the like, including the corresponding acid halides and lower aliphatic esters. A mole ratio of maleic anhydride to polyalkenyl component in the reaction mixture may vary widely. Accordingly, the mole ratio may vary from about 5:1 to about 1.5, for example from about 3:1 to about 1:3, and as a further example, the maleic anhydride may be used in stoichiometric excess to force the reaction to completion. The unreacted maleic anhydride may be removed by vacuum distillation.

Any of numerous amines can be used to prepare the polyalkenyl or hydrocarbyl-substituted succinimide dispersant, provided the amines are polyamines containing at least two nitrogen atoms. Non-limiting exemplary polyamines may include aminoguanidine bicarbonate (AGBC), diethylene triamine (DETA), triethylene tetramine (TETA), tetraethylene pentamine (TEPA), pentaethylene hexamine (PEHA) and heavy polyamines. A heavy polyamine may comprise a mixture of polyalkylene polyamines having small amounts of lower polyamine oligomers such as TEPA and PEHA, but primarily oligomers having seven or more nitrogen atoms, two or more primary amines per molecule, and more extensive branching than conventional polyamine mixtures. Additional non-limiting polyamines which may be used to prepare the hydrocarbyl-substituted succinimide dispersant are disclosed in U.S. Pat. No. 6,548,458, the disclosure of which is incorporated herein by reference in its entirety. In an embodiment of the disclosure, the polyamine may be selected from tetraethylene pentamine (TEPA).

In an embodiment, the dispersant derivative may be derived compounds of formula:



wherein n represents 0 or an integer of from 1 to 5, and  $\text{R}^2$  is a hydrocarbyl substituent as defined above. In an embodiment, n is 3 and  $\text{R}^2$  is a polyisobutylene substituent, such as that derived from polyisobutylenes having at least about 60%, such as about 70% to about 90% and above, terminal

vinylidene content. Compounds of formula (IV) may be the reaction product of a hydrocarbyl-substituted succinic anhydride, such as a polyisobutylene succinic anhydride (PIBSA), and a polyamine, for example tetraethylene pentamine (TEPA).

The foregoing dispersant may have a molar ratio of (A) polyisobutylene-substituted succinic anhydride to (B) polyamine in the range 4:3 to 1:10 in the dispersant. A particularly useful dispersant contains polyisobutylene group of the polyisobutylene-substituted succinic anhydride having a number average molecular weight (Mn) in the range of from about 500 to 850 as determined by GPC and a (B) polyamine having a general formula  $H_2N(CH_2)_m-[NH(CH_2)_m]_n-NH_2$ , wherein m is in the range from 2 to 4 and n is in the range of from 1 to 3.

The amine moiety of the mono-succinimide dispersant described above may be further reacted with an acidic compound containing two or more pyrrole groups. For example, the acidic compound may contain four pyrrole groups in a cycloaromatic ring. The each of the pyrrole groups in the acid compound may be substituted with a  $C_1$  to  $C_4$  alkyl group, a  $C_1$  to  $C_4$  alkenyl group. Such compounds may include linear and cyclic tetrapyrroles such as a porphyrin compound, typically a porphyrin acid or anhydride compound, specifically protoporphyrin IX having the following formula:



The amount of mono-succinimide dispersant reacted with the porphyrin compound may range from about 0.5:1 to about 2:1 on a molar ratio. A desirable amount of porphyrin compound to dispersant may range from about 0.8:1 to about 1.2:1. The exact nature of the reaction product is not readily determinable but may be a mixture of capped dispersants having a porphyrin moiety attached to a primary nitrogen atom and uncapped dispersants containing one or more porphyrin moieties attached to secondary nitrogen atoms, or a mixture of capped and uncapped dispersants. The amount of porphyrin reacted dispersant that may be used in a lubricant composition may range from about 0.5 to about 5.0 percent by weight based on a total weight of the lubricant composition.

#### Phosphorus-Based Antiwear Agents

The phosphorus-based wear preventative may comprise a metal dihydrocarbyl dithiophosphate compound, such as but not limited to a zinc dihydrocarbyl dithiophosphate compound. Suitable metal dihydrocarbyl dithiophosphates may comprise dihydrocarbyl dithiophosphate metal salts wherein the metal may be an alkali or alkaline earth metal, or aluminum, lead, tin, molybdenum, manganese, nickel, copper, or zinc.

Dihydrocarbyl dithiophosphate metal salts may be prepared in accordance with known techniques by first forming a dihydrocarbyl dithiophosphoric acid (DDPA), usually by reaction of one or more alcohol or a phenol with  $P_2S_5$  and then neutralizing the formed DDPA with a metal compound. For example, a dithiophosphoric acid may be made by reacting mixtures of primary and secondary alcohols. Alternatively, multiple dithiophosphoric acids can be prepared where the hydrocarbyl groups on one are entirely secondary in character and the hydrocarbyl groups on the others are entirely primary in character. To make the metal salt, any basic or neutral metal compound could be used but the oxides, hydroxides and carbonates are most generally employed. Commercial additives frequently contain an excess of metal due to the use of an excess of the basic metal compound in the neutralization reaction.

The zinc dihydrocarbyl dithiophosphates (ZDDP) are oil soluble salts of dihydrocarbyl dithiophosphoric acids and may be represented by the following formula:



wherein R and R' may be the same or different hydrocarbyl radicals containing from 1 to 18, for example 2 to 12, carbon atoms and including radicals such as alkyl, alkenyl, aryl, arylalkyl, alkaryl, and cycloaliphatic radicals. R and R' groups may be alkyl groups of 2 to 8 carbon atoms. Thus, the radicals may, for example, be ethyl, n-propyl, i-propyl, n-butyl, i-butyl, sec-butyl, amyl, n-hexyl, i-hexyl, n-octyl, decyl, dodecyl, octadecyl, 2-ethylhexyl, phenyl, butylphenyl, cyclohexyl, methylecyclopentyl, propenyl, butenyl. In order to obtain oil solubility, the total number of carbon atoms (i.e., R and R') in the dithiophosphoric acid will generally be about 5 or greater. The zinc dihydrocarbyl dithiophosphate can therefore comprise zinc dialkyl dithiophosphates.

Other suitable components that may be utilized as the phosphorus-based wear preventative include any suitable organophosphorus compound, such as but not limited to, phosphates, thiophosphates, di-thiophosphates, phosphites, and salts thereof and phosphonates. Suitable examples are tricresyl phosphate (TCP), di-alkyl phosphite (e.g., dibutyl hydrogen phosphate), and amyl acid phosphate.

Another suitable component is a phosphorylated succinimide such as a completed reaction product from a reaction between a hydrocarbyl substituted succinic acylating agent and a polyamine combined with a phosphorus source, such as inorganic or organic phosphorus acid or ester. Further, it may comprise compounds wherein the product may have amide, amidine, and/or salt linkages in addition to the imide linkage of the type that results from the reaction of a primary amino group and an anhydride moiety.

The phosphorus-based wear preventative may be present in a lubricating composition in an amount sufficient to provide from about 200 to about 2000 ppm phosphorus. As a further example, the phosphorus-based wear preventative may be present in a lubricating composition in an amount sufficient to provide from about 500 to about 800 ppm phosphorus.

The phosphorus-based wear preventative may be present in a lubricating composition in an amount sufficient to provide a ratio of alkali and/or alkaline earth metal content (ppm) based on the total amount of alkali and/or alkaline earth metal in the lubricating composition to phosphorus content (ppm) based

on the total amount of phosphorus in the lubricating composition of from about 1.6 to about 3.0 (ppm/ppm).

#### Friction Modifiers

Embodiments of the present disclosure may include one or more friction modifiers. Suitable friction modifiers may comprise metal containing and metal-free friction modifiers and may include, but are not limited to, imidazolines, amides, amines, succinimides, alkoxylated amines, alkoxylated ether amines, amine oxides, amidoamines, nitriles, betaines, quaternary amines, imines, amine salts, amino guanadine, alkanolamides, phosphonates, metal-containing compounds, glycerol esters, and the like.

Suitable friction modifiers may contain hydrocarbyl groups that are selected from straight chain, branched chain, or aromatic hydrocarbyl groups or admixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms and may be saturated or unsaturated.

Aminic friction modifiers may include amides of polyamines. Such compounds can have hydrocarbyl groups that are linear, either saturated or unsaturated, or a mixture thereof and may contain from about 12 to about 25 carbon atoms.

Further examples of suitable friction modifiers include alkoxylated amines and alkoxylated ether amines. Such compounds may have hydrocarbyl groups that are linear, either saturated, unsaturated, or a mixture thereof. They may contain from about 12 to about 25 carbon atoms. Examples include ethoxylated amines and ethoxylated ether amines.

The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291, herein incorporated by reference.

Other suitable friction modifiers may include an organic, ashless (metal-free), nitrogen-free organic friction modifier. Such friction modifiers may include esters formed by reacting carboxylic acids and anhydrides with alkanols. Other useful friction modifiers generally include a polar terminal group (e.g. carboxyl or hydroxyl) covalently bonded to an oleophilic hydrocarbon chain. Esters of carboxylic acids and anhydrides with alkanols are described in U.S. Pat. No. 4,702,850. Another example of an organic ashless nitrogen-free friction modifier is known generally as glycerol monocoleate (GMO) which may contain mono- and diesters of oleic acid. Other suitable friction modifiers are described in U.S. Pat. No. 6,723,685, herein incorporated by reference. The ashless friction modifier may be present in the lubricant composition in an amount ranging from about 0.1 to about 0.4 percent by weight based on a total weight of the lubricant composition.

Suitable friction modifiers may also include one or more molybdenum compounds. The molybdenum compound may be selected from the group consisting of molybdenum dithiocarbamates (MoDTC), molybdenum dithiophosphates, molybdenum dithiophosphinates, molybdenum xanthates, molybdenum thioxanthates, molybdenum sulfides, a tri-nuclear organo-molybdenum compound, molybdenum/amine complexes, and mixtures thereof.

Additionally, the molybdenum compound may be an acidic molybdenum compound. Included are molybdic acid, ammonium molybdate, sodium molybdate, potassium molybdate, and other alkaline metal molybdates and other molybdenum salts, e.g., hydrogen sodium molybdate,  $\text{MoOCl}_4$ ,  $\text{MoO}_2\text{Br}_2$ ,  $\text{Mo}_2\text{O}_3\text{Cl}_6$ , molybdenum trioxide or

similar acidic molybdenum compounds. Alternatively, the compositions can be provided with molybdenum by molybdenum/sulfur complexes of basic nitrogen compounds as described, for example, in U.S. Pat. Nos. 4,263,152; 4,285,822; 4,283,295; 4,272,387; 4,265,773; 4,261,843; 4,259,195 and 4,259,194; and WO 94/06897.

Suitable molybdenum dithiocarbamates may be represented by the formula:

10



15

where  $R_1$ ,  $R_2$ ,  $R_3$ , and  $R_4$  each independently represent a hydrogen atom, a  $C_1$  to  $C_{20}$  alkyl group, a  $C_6$  to  $C_{20}$  cycloalkyl, aryl, alkylaryl, or aralkyl group, or a  $C_3$  to  $C_{20}$  hydrocarbyl group containing an ester, ether, alcohol, or carboxyl group; and  $X_1$ ,  $X_2$ ,  $Y_1$ , and  $Y_2$  each independently represent a sulfur or oxygen atom.

Examples of suitable groups for each of  $R_1$ ,  $R_2$ ,  $R_3$ , and  $R_4$  include 2-ethylhexyl, nonylphenyl, methyl, ethyl, n-propyl, iso-propyl, n-butyl, t-butyl, n-hexyl, n-octyl, nonyl, decyl, dodecyl, tridecyl, lauryl, oleyl, linoleyl, cyclohexyl and phenylmethyl.  $R_1$  to  $R_4$  may each have  $C_6$  to  $C_{18}$  alkyl groups.  $X_1$  and  $X_2$  may be the same, and  $Y_1$  and  $Y_2$  may be the same.  $X_1$  and  $X_2$  may both comprise sulfur atoms, and  $Y_1$  and  $Y_2$  may both comprise oxygen atoms.

Further examples of molybdenum dithiocarbamates include  $C_6$ - $C_{18}$  dialkyl or diaryldithiocarbamates, or alkyl-aryldithiocarbamates such as dibutyl-, diethyl-di-(2-ethylhexyl)-, dilauryl-, dioleyl-, and dicyclohexyl-dithiocarbamate.

Another class of suitable organo-molybdenum compounds are trinuclear molybdenum compounds, such as those of the formula  $\text{Mo}_3\text{S}_k\text{L}_n\text{Q}_z$  and mixtures thereof, wherein L represents independently selected ligands having organo groups with a sufficient number of carbon atoms to render the compound soluble or dispersible in the oil, n is from 1 to 4, k varies from 4 through 7, Q is selected from the group of neutral electron donating compounds such as water, amines, alcohols, phosphines, and ethers, and z ranges from 0 to 5 and includes non-stoichiometric values. At least 21 total carbon atoms may be present among all the ligands' organo groups, such as at least 25, at least 30, or at least 35 carbon atoms. Additional suitable molybdenum compounds are described in U.S. Pat. No. 6,723,685, herein incorporated by reference.

The molybdenum compound may be present in a fully formulated crankcase lubricant in an amount to provide about 5 ppm to 200 ppm molybdenum. As a further example, the molybdenum compound may be present in an amount to provide about 50 to 100 ppm molybdenum.

Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent). The use of an additive concentrate may take advantage of the mutual compatibility afforded by the combination of ingredients when in the form of an additive concentrate. Also, the use of a concentrate may reduce blending time and may lessen the possibility of blending errors.

## 11

The present disclosure provides novel lubricating oil blends specifically formulated for use as automotive crankcase lubricants. Embodiments of the present disclosure may provide lubricating oils suitable for crankcase applications and having improvements in the following characteristics: antioxidant, antiwear performance, rust inhibition, fuel economy, water tolerance, air entrainment, and foam reducing properties.

## Anti-Foam Agents

In some embodiments, a foam inhibitor may form another component suitable for use in the compositions. Foam inhibitors may be selected from silicones, polyacrylates, and the like. The amount of antifoam agent in the crankcase lubricant formulations described herein may range from about 0.001 wt % to about 0.1 wt % based on the total weight of the formulation. As a further example, antifoam agent may be present in an amount from about 0.004 wt % to about 0.008 wt %.

## Oxidation Inhibitor Components

Oxidation inhibitors or antioxidants reduce the tendency of base stocks to deteriorate in service which deterioration can be evidenced by the products of oxidation such as sludge and varnish-like deposits that deposit on metal surfaces and by viscosity growth of the finished lubricant. Such oxidation inhibitors include hindered phenols, sulfurized hindered phenols, alkaline earth metal salts of alkylphenolthioesters having C<sub>5</sub> to C<sub>12</sub> alkyl side chains, sulfurized alkylphenols, metal salts of either sulfurized or nonsulfurized alkylphenols, for example calcium nonylphenol sulfide, ashless oil soluble phenates and sulfurized phenates, phosphosulfurized or sulfurized hydrocarbons, phosphorus esters, metal thiocarbamates, and oil soluble copper compounds as described in U.S. Pat. No. 4,867,890.

Other antioxidants that may be used include sterically hindered phenols and esters thereof, diarylamines, alkylated phenothiazines, sulfurized compounds, and ashless dialkylthiocarbamates. Non-limiting examples of sterically hindered phenols include, but are not limited to, 2,6-di-tertiary butylphenol, 2,6 di-tertiary butyl methylphenol, 4-ethyl-2,6-di-tertiary butylphenol, 4-propyl-2,6-di-tertiary butylphenol, 4-butyl-2,6-di-tertiary butylphenol, 4-pentyl-2,6-di-tertiary butylphenol, 4-hexyl-2,6-di-tertiary butylphenol, 4-heptyl-2,6-di-tertiary butylphenol, 4-(2-ethylhexyl)-2,6-di-tertiary butylphenol, 4-octyl-2,6-di-tertiary butylphenol, 4-nonyl-2,6-di-tertiary butylphenol, 4-decyl-2,6-di-tertiary butylphenol, 4-undecyl-2,6-di-tertiary butylphenol, 4-dodecyl-2,6-di-tertiary butylphenol, methylene bridged sterically hindered phenols including but not limited to 4,4-methylenebis(6-tert-butyl-o-cresol), 4,4-methylenebis(2-tert-amyl-o-cresol), 2,2-methylenebis(4-methyl-6-tert-butylphenol), 4,4-methylenebis(2,6-di-tert-butylphenol) and mixtures thereof as described in U.S. Publication No. 2004/0266630.

Diarylamine antioxidants include, but are not limited to diarylamines having the formula:



wherein R' and R" each independently represents a substituted or unsubstituted aryl group having from 6 to 30 carbon atoms. Illustrative of substituents for the aryl group include aliphatic hydrocarbon groups such as alkyl having from 1 to 30 carbon atoms, hydroxy groups, halogen radicals, carboxylic acid or ester groups, or nitro groups.

The aryl group is preferably substituted or unsubstituted phenyl or naphthyl, particularly wherein one or both of the

## 12

aryl groups are substituted with at least one alkyl having from 4 to 30 carbon atoms, preferably from 4 to 18 carbon atoms, most preferably from 4 to 9 carbon atoms. It is preferred that one or both aryl groups be substituted, e.g. mono-alkylated diphenylamine, di-alkylated diphenylamine, or mixtures of mono- and di-alkylated diphenylamines.

The diarylamines may be of a structure containing more than one nitrogen atom in the molecule. Thus the diarylamine may contain at least two nitrogen atoms wherein at least one nitrogen atom has two aryl groups attached thereto, e.g. as in the case of various diamines having a secondary nitrogen atom as well as two aryls on one of the nitrogen atoms.

Examples of diarylamines that may be used include, but are not limited to: diphenylamine; various alkylated diphenylamines; 3-hydroxydiphenylamine; N-phenyl-1,2-phenylenediamine; N-phenyl-1,4-phenylenediamine; monobutylidiphenyl-amine; dibutylidiphenylamine; monoocetylidiphenylamine; dioctylidiphenylamine; monononylidiphenylamine; dinonylidiphenylamine; monotetradecylidiphenylamine; ditetradecylidiphenylamine, phenyl-alpha-naphthylamine; monoocetyl phenyl-alpha-naphthylamine; phenyl-beta-naphthylamine; monoheptylidiphenylamine; diheptyl-diphenylamine; p-oriented styrenated diphenylamine; mixed butyloctyldiphenylamine; and mixed octylstyryldiphenylamine.

The sulfur containing antioxidants include, but are not limited to, sulfurized olefins that are characterized by the type of olefin used in their production and the final sulfur content of the antioxidant. High molecular weight olefins, i.e. those olefins having an average molecular weight of 168 to 351 g/mole, are preferred. Examples of olefins that may be used include alpha-olefins, isomerized alpha-olefins, branched olefins, cyclic olefins, and combinations of these.

Alpha-olefins include, but are not limited to, any C<sub>4</sub> to C<sub>25</sub> alpha-olefins. Alpha-olefins may be isomerized before the sulfurization reaction or during the sulfurization reaction. Structural and/or conformational isomers of the alpha olefin that contain internal double bonds and/or branching may also be used. For example, isobutylene is a branched olefin counterpart of the alpha-olefin 1-butene.

Sulfur sources that may be used in the sulfurization reaction of olefins include: elemental sulfur, sulfur monochloride, sulfur dichloride, sodium sulfide, sodium polysulfide, and mixtures of these added together or at different stages of the sulfurization process.

Unsaturated oils, because of their unsaturation, may also be sulfurized and used as an antioxidant. Examples of oils or fats that may be used include corn oil, canola oil, cottonseed oil, grapeseed oil, olive oil, palm oil, peanut oil, coconut oil, rapeseed oil, safflower seed oil, sesame seed oil, soyabean oil, sunflower seed oil, tallow, and combinations of these.

The amount of sulfurized olefin or sulfurized fatty oil delivered to the finished lubricant is based on the sulfur content of the sulfurized olefin or fatty oil and the desired level of sulfur to be delivered to the finished lubricant. For example, a sulfurized fatty oil or olefin containing 20 weight % sulfur, when added to the finished lubricant at a 1.0 weight % treat level, will deliver 2000 ppm of sulfur to the finished lubricant.

A sulfurized fatty oil or olefin containing 10 weight % sulfur, when added to the finished lubricant at a 1.0 weight % treat level, will deliver 1000 ppm sulfur to the finished lubricant. It is desirable that the sulfurized olefin or sulfurized fatty oil to deliver between 200 ppm and 2000 ppm sulfur to the finished lubricant.

In general terms, a suitable crankcase lubricant may include additive components in the ranges listed in the following table.

TABLE 2

| Component                                   | Wt. %<br>(Broad) | Wt. %<br>(Typical) |
|---------------------------------------------|------------------|--------------------|
| Dispersant                                  | 0.5-10.0         | 1.0-5.0            |
| Antioxidant system                          | 0-5.0            | 0.01-3.0           |
| Metal Detergents                            | 0.1-15.0         | 0.2-8.0            |
| Corrosion Inhibitor                         | 0-5.0            | 0-2.0              |
| Metal dihydrocarbyl dithiophosphate         | 0.1-6.0          | 0.1-4.0            |
| Ash-free amine phosphate salt               | 0.0-6.0          | 0.0-4.0            |
| Antifoaming agent                           | 0-5.0            | 0.001-0.15         |
| Supplemental antiwear agents                | 0-1.0            | 0-0.8              |
| Pour point depressant                       | 0.01-5.0         | 0.01-1.5           |
| Viscosity modifier                          | 0.01-20.00       | 0.25-10.0          |
| Supplemental friction modifier <sup>1</sup> | 0-2.0            | 0.1-1.0            |
| Base oil                                    | Balance          | Balance            |
| Total                                       | 100              | 100                |

In order to demonstrate the benefits and advantages of lubricant compositions according to the disclosure, the following non-limiting examples are provided.

### EXAMPLES

#### Dispersant/Porphyrin Reaction Product

A dispersant/porphyrin reaction product was made by combining 5 grams of 50 wt. % active 2100 molecular weight polyisobutylene-substituted succinimide dispersant with 0.456 grams of protoporphyrin IX in a 10 mL reaction vessel containing a magnetic stir bar. The reaction mixture was stirred and heated to 180° C. under one atmosphere of nitrogen gas pressure. Once the temperature was reached, the reaction mixture was held for 4 hours with stirring. After vacuum stripping to remove any water, the material was filtered.

In order to demonstrate the effectiveness of the dispersant/porphyrin reaction product made by the foregoing procedure, lubricant formulations containing conventional dispersants and the dispersant/porphyrin reaction product were tested in a Thermo-oxidation Engine Oil Simulation Test (TEOST MHT-4). The TEOST MHT-4 test is a standard lubricant industry test (ASTM D-7097) that evaluates the oxidation and carbonaceous deposit-forming characteristics of engine oils. The test is designed to simulate high temperature (285° C.) deposits in the piston ring belt area of engines. The focus of the test is to obtain the weight of the deposit formed on a resistively-heated depositor rod held within a casing as bulk oil is flowed past it at a rate of 0.25 g/minute. The temperature of the rod is controlled by a thermocouple. The use of a catalyst consisting of 3/2/1 ratio of iron, lead, and tin is used to increase oxidation stress on the oil. The oxidation in the test is measured in terms of the mass of the deposits that are formed on the rod and on a filter in the instrument used for the test.

In each of the following examples, a fully treated lubricant composition was top treated with Prior Art Dispersant 1 (a mono-succinimide dispersant), Prior Art Dispersant 2 (a bis-succinimide dispersant) and Dispersant 3 (Dispersant 1 reacted with protoporphyrin IX according to the foregoing example). The results are contained in the attached table.

| 5  | Dispersant | Wt. % | Rod           | Filter        | Total         | TBN (mg KOH/g) | TBN/wt. % |
|----|------------|-------|---------------|---------------|---------------|----------------|-----------|
|    |            |       | Deposits (mg) | deposits (mg) | deposits (mg) |                |           |
| 10 | 1          | 1.6   | 16.1          | 0             | 16.1          | 8.78           | 5.5       |
|    | 2          | 2.4   | 14.2          | 4.8           | 19.0          | 9.06           | 3.8       |
|    | 3          | 1.2   | 5.3           | 0             | 5.3           | 8.53           | 7.1       |

10 As shown by the foregoing examples, Dispersant 3 provides significantly better total deposits and rod deposits than Dispersants 1 and 2. The results was surprising and totally unexpected, particularly in view of the use of significantly less Dispersant 3 than Dispersant 1 or Dispersant 2 in the lubricant composition.

15 At numerous places throughout this specification, reference has been made to a number of U.S. Patents. All such cited documents are expressly incorporated in full into this disclosure as if fully set forth herein.

20 Other embodiments of the present disclosure will be apparent to those skilled in the art from consideration of the specification and practice of the embodiments disclosed herein. As used throughout the specification and claims, "a" and/or "an" may refer to one or more than one. Unless otherwise indicated, all numbers expressing quantities of ingredients, properties such as molecular weight, percent, ratio, reaction conditions, and so forth used in the specification and claims are to be understood as being modified in all instances by the term "about." Accordingly, unless indicated to the contrary, the

25 numerical parameters set forth in the specification and claims are approximations that may vary depending upon the desired properties sought to be obtained by the present invention. At the very least, and not as an attempt to limit the application of the doctrine of equivalents to the scope of the claims, each 30 numerical parameter should at least be construed in light of the number of reported significant digits and by applying ordinary rounding techniques. Notwithstanding that the numerical ranges and parameters setting forth the broad scope of the invention are approximations, the numerical 35 values set forth in the specific examples are reported as precisely as possible. Any numerical value, however, inherently contains certain errors necessarily resulting from the standard deviation found in their respective testing measurements. It is intended that the specification and examples be considered as 40 exemplary only, with a true scope and spirit of the invention being indicated by the following claims.

45 The foregoing embodiments are susceptible to considerable variation in practice. Accordingly, the embodiments are not intended to be limited to the specific exemplifications set forth hereinabove. Rather, the foregoing embodiments are within the spirit and scope of the appended claims, including the equivalents thereof available as a matter of law.

The patentees do not intend to dedicate any disclosed 50 embodiments to the public, and to the extent any disclosed modifications or alterations may not literally fall within the scope of the claims, they are considered to be part hereof under the doctrine of equivalents.

What is claimed is:

1. A crankcase lubricant composition comprising a base oil and a reaction product of mono-succinimide dispersant and an acidic compound containing two or more pyrrole groups.
2. The crankcase lubricant composition of claim 1, wherein the acidic compound comprises 4 pyrrole groups in cycloaromatic ring.
3. The crankcase lubricant composition of claim 1, wherein the acidic compound comprises a porphyrin acid or anhydride.

## 15

4. The crankcase lubricant composition of claim 1, wherein the acidic compound comprises protoporphyrin IX.

5. The crankcase lubricant composition of claim 1, wherein the lubricant composition comprises from about 0.5 to about 5 percent by weight of the reaction product based on a total weight of the lubricant composition.

6. A method for improving the soot or sludge handling capability of a crankcase lubricant for an engine composition comprising formulating a lubricant composition for the engine with a base oil and an amount of a reaction product of mono-succinimide dispersant and an acidic compound containing at least two pyrrole groups, wherein the succinimide dispersant comprises an amine moiety having at least two nitrogen atoms.

7. The method of claim 6, wherein the acidic compound comprises 4 pyrrole groups in cycloaromatic ring.

8. The method of claim 6, wherein the acidic compound comprises a porphyrin acid or anhydride.

9. The method of claim 6, wherein the acidic compound comprises protoporphyrin IX.

10. The method of claim 6, wherein the lubricant composition comprises from about 0.5 to about 5 percent by weight of the reaction product based on a total weight of the lubricant composition.

11. The method of claim 6, wherein the lubricant composition further comprises a metal detergent, wherein the metal detergent comprises a detergent selected from the group consisting of overbased calcium sulfonate, overbased magnesium sulfonate, overbased calcium phenate, overbased magnesium phenate, and mixtures thereof.

## 16

12. A method for operating an engine comprising; formulating a crankcase lubricant for the engine comprising a base oil and a lubricant additive package comprising an amount of a reaction product of mono-succinimide dispersant and an acidic compound containing at least two pyrrole groups, wherein the succinimide dispersant comprises an amine moiety having at least two nitrogen atoms; and operating the engine with the crankcase lubricant.

13. The method of claim 11, wherein the acidic compound comprises 4 pyrrole groups in cycloaromatic ring.

14. The method of claim 11, wherein the acidic compound comprises a porphyrin acid or anhydride.

15. The method of claim 11, wherein the acidic compound comprises protoporphyrin IX.

16. The method of claim 11, further comprising a metal detergent, wherein the metal detergent comprises a detergent selected from the group consisting of overbased calcium sulfonate, overbased magnesium sulfonate, overbased calcium phenate, and overbased magnesium phenate.

17. The method of claim 11, wherein the amount of reaction product in the lubricant composition may range from about 0.5 to about 5 percent by weight of the total weight of the lubricant composition.

18. The method of claim 11, wherein the engine comprises a heavy duty diesel engine.

19. The method of claim 11, wherein the engine comprises a gasoline engine.

\* \* \* \* \*